

May 12, 1942.

R. ETZKORN

2,282,466

FIBROUS MATERIAL

Filed Feb. 4, 1938

Fig. 1



Fig. 2



Inventor:  
Rudolf Etzkorn

By E. F. Mandeville  
Atty

## UNITED STATES PATENT OFFICE

2,282,466

## FIBROUS MATERIAL

Rudolf Etzkorn, Murg, Baden, Germany

Application February 4, 1938, Serial No. 188,764  
In Germany February 9, 1937

3 Claims. (Cl. 252—14)

This invention relates to a fibrous material for use in stuffing boxes and the like and to a process of manufacturing such packing material.

It is the object of this invention to provide means in the packing material for reducing the wear of the stuffing boxes or other machine parts to be packed by the said material.

Another object of the present invention is to incorporate lubricating or protective substances in fibrous carrier materials.

Still another object of my invention is to increase the duration of the packing material and to improve its resistability against active substances.

Further objects and particulars of my invention will be clear from the following detailed description of some examples of my novel packing material in connection with the accompanying drawing, showing by way of example and schematically in Fig. 1 an axial section of a stuffing box provided with my novel packing material and in Fig. 2 a cross-section of one capillary fibre of my novel packing material, on a greatly enlarged scale.

As will be seen from Fig. 1, a rotary shaft or reciprocating rod 1 is packed in normal manner by a stuffing box comprising a casing 2 and a press-member 4 which can be moved into the inner cylindrical bore of the casing 2 by means of screws 8. Located in the annular space between the shaft 1 and the inner walls of the casing 2, in the manner known per se, is the packing material comprising cords 3 of a square cross section composed of a plurality of threads 1. Each thread 1 in turn consists of a great number, for instance, 1000 to 10,000 or more capillary fibres which according to my invention contain a lubricating substance, such as, for instance, oil, fat, tallow, wax or graphite, extending throughout the fibrous material, in a finely distributed form.

Fig. 2 shows, in a greatly enlarged cross-sectional view, a single capillary fibre, consisting of small particles 5 of lubricating substances and a skeleton material 6 consisting, for instance, of regenerated cellulose.

The manufacture of the artificial fibrous material is based on the solution of cellulose or cellulose compounds in suitable solvents or soluble chemical compounds. This spinning material is then introduced into a gaseous or liquid precipitating bath through a number of fine orifices the width of which depends upon the kind of spinning process employed. The cellulose or cellulose compound is thereby precipitated in the

form of a thread or filament which can be worked up into a textile fabric. If now one or more of the aforesaid protective substances which are most suitable for incorporation in soft packings, for example finely divided graphite or graphite and oil, are mixed with the spinning liquid in a quantity which is so great that the amount of cellulose or cellulose compound present is just sufficient to form a thread which still has sufficient strength to be worked further, there is then obtained an artificial fibrous material of which the smallest particles of its structure are filled and combined with the protective agent. The method of manufacturing the material is not limited in any way as regards the chemical process adapted. Useful threads can be obtained both by the viscose and super-ammonia process; the nitrate and acetate processes are also suitable and any spinning process which allows the protective substances to be added in sufficiently large quantity to the spinning solution may be employed. The threads or fibres thus obtained may be combined to a packing material in any suitable manner. I contemplate, for example, to produce the packing of many short threads or fibres felted together in the form of a substance similar to lap. According to a preferred modification the said short artificial fibres may be spun in the form of continuous threads as known in the textile industries and be used in the form of cords, strings, twines or the like obtained by twisting such threads. Also, a packing may be made of slubbings or rovings comprising many parallelly running practically endless fibres. The threads may have a round or circular cross-section, such as obtained by pressing or squeezing a solution through round nozzles and then solidifying the fibre. By way of alternative, the single fibre may have an oval or rectangular cross-section so as to form a narrow band. Such band-shaped fibres may be produced by pressing or squeezing a spinning solution containing the lubricant through slot-shaped nozzles or by cutting a foil obtained from such a solution into narrow strips. The spinning process per se is the same as known in the manufacture of artificial silk and therefore it will not be necessary to describe this process in a greater detail.

The thickness of the single fibre or capillary thread in which the lubricant or lubricants or a mixture of lubricants are embodied may be varied within wide limits. For example, the single thread may have a thickness of 1-10 denier (that is to say 9000 meters of such a fibre would have

a weight of 1-10 grams) or I may use substantially thicker fibres having, for example, a diameter of 0.2 to 0.5 mm. and more.

The size of the particles of oil, fat, graphite or like lubricants depends on the thickness of the capillary fibre and the manner in which the same is produced.

Very thin fibres containing relatively coarse embeddings can be produced, for instance, by squeezing a solution of cellulose acetate in acetone, containing the finely distributed lubricants, through nozzles and attenuating the fibre or sliver so formed, before its solidification, by strongly drawing it out in the manner known per se in the spinning art. In this manner clogging or choking of the nozzles can be avoided even with coarse lubricant particles embedded in the fibre.

The quantity of oily substances, such as oil or graphite incorporated in the single fibre depends on the desired oiliness. The maximum amount will be determined by the fact that the percentage of the substance forming the fibre, such as regenerated cellulose or cellulose acetate or the like has to be sufficiently high as to obtain a cohering fibre. Generally, in order to ensure a satisfactory lubricating effect, the percentage of lubricating substances will not be made less than 10% of the weight of the complete fibre. I have found that a percentage of 15 or preferably of 25-60 percent of graphite is very favorable, although it is possible to incorporate even higher percentages of lubricating material into the fibre mass.

Where graphite is used as a lubricator, I use the same preferably in a colloidal form, for instance in the form of deflocculated Acheson graphite. Where it is intended to incorporate an oil besides a solid lubricating substance, such as graphite, the same may be incorporated in the solution of the fibre-forming substance besides the solid substance. A very favourable lubricating effect or oiliness is obtained, if the solid substance is first finely distributed or dispersed in the oil and the suspension thus obtained is then combined with or admixed to, the spinning solution. For example, the suspension of graphite of the kind known under the trade name "Oildag" may be finely dispersed in a cellulose solution such as viscose, by intimate stirring. This cellulose solution, when formed into fibres of round or approximately rectangular cross-

section, forms a fibrous substance in which small particles of the said suspension are dispersed throughout the cellulose.

The use of the fibrous material described as a soft packing not only has the great advantage that the wear on the packed machine parts is reduced to a minimum, but it has also been found that this packing is resistant to the action of almost all substances employed in industry. An examination of the material has also proved, for example when graphite is employed, that particles of graphite are set free very easily by friction, the result of which is that the coefficient of friction is very small. The extremely small wear on the packed machine parts may be explained primarily by the fact that the friction is for the most part taken up by the particles of protective material, for example flakes of graphite, which are embedded in the basic artificial fabric, while, on the other hand, the artificial fibrous material which acts as the carrier for the protective particles contains an extremely small proportion of mineral constituents having a grinding effect, as can be proved by the ash content of the material.

While I have herein shown and described certain preferred embodiments of my invention, I wish it to be understood that I do not confine myself to all the precise details herein set forth by way of illustration, as modification and variation may be made without departing from the spirit of the invention or exceeding the scope of the appended claims.

I claim:

35 1. In a stuffing box a packing comprising artificial fibers and particles of graphite incorporated in and finely distributed throughout the said fibers, the percentage of graphite being above 10% of the weight of the complete fiber.

40 2. In a stuffing box a packing comprising artificial fibers and particles of graphite incorporated in and finely distributed throughout the said fibers, the percentage of graphite being 25-60% of the weight of the complete fiber.

45 3. In a stuffing box, a packing comprising artificial fibers and particles of graphite as well as of a liquid lubricant incorporated and finely distributed throughout the said fibers, the percentage of graphite being 25-60% of the weight of the complete fiber.

RUDOLF ETZKORN.